

(No Model.)

E. W. RICE, Jr.  
COMMUTATOR BRUSH.

No. 447,352.

Patented Mar. 3, 1891.



WITNESSES  
John F. McDonald  
A. C. Dine

INVENTOR  
Edwin W. Rice Jr  
by Bradley Knight  
Attest.

# UNITED STATES PATENT OFFICE.

EDWIN WILBUR RICE, JR., OF LYNN, MASSACHUSETTS, ASSIGNOR TO THE THOMSON-HOUSTON ELECTRIC COMPANY, OF CONNECTICUT.

## COMMUTATOR-BRUSH.

SPECIFICATION forming part of Letters Patent No. 447,352, dated March 3, 1891.

Application filed November 28, 1890. Serial No. 372,859. (No model.)

To all whom it may concern:

Be it known that I, EDWIN WILBUR RICE, Jr., a citizen of the United States, residing at Lynn, county of Essex, and State of Massachusetts, have invented a certain new and useful Improvement in Commutator-Brushes, of which the following is a specification.

My present invention relates to carbon commutator-brushes for dynamo-electric machines; and it consists in providing such a brush with a coating of metal gradually decreasing in thickness toward its wearing-surface, for I have found that such a coating gives the brush all the advantages gained by the metal coating of brushes now in use, and, furthermore, avoids peeling of the coating from the carbon with the evil results incident thereto, which have proved heretofore a serious defect.

It has been customary to cover a carbon brush with a coating of copper of uniform thickness, as indicated in Figures 4 and 5 of the accompanying drawings, for securing a comparatively high degree of conductivity and avoiding heating. Upon using these brushes, however, it is found that the lower portions of the coating will peel off from the carbon, forming a rough jagged wearing-edge, liable to cause short circuits in the machine, poor contacts, and to interfere with freedom of play of the brush in its holder. This peeling is what I now aim to avoid, and I have found that it can be done by gradually decreasing the thickness of the metal coating, so that at the wearing-surface of the brush the coating is very thin, practically no more than a metal film. It will then wear off smoothly and does not readily become caught, thereby stripping or peeling the coating.

These improvements are illustrated in the accompanying drawings, wherein—

Figs. 1, 2, and 3 are respectively sections taken through one of my improved brushes with the metal coating applied in slightly-modified ways; and Figs. 4 and 5 illustrate in perspective and in section an old form of commutator-brush upon which my invention is an improvement.

In the drawings, A represents a carbon commutator-brush similar to those now in use,

and B the metal coating. In Fig. 1 this coating tapers uniformly from one end of the brush nearly down to its wearing-surface, while in Fig. 2 the coating is of uniform thickness to a point at about the middle of the brush, and from there on tapers down, so that the thickness of the coating is gradually decreased, terminating at a, as before, in a mere film. Fig. 3 shows a similar coating of gradually-decreasing thickness; but in this modification the coating resembles a succession of layers of varying and gradually-decreasing thickness. This arrangement, while the same in idea, is not considered so good as that in either of the preceding figures, for the increase in conductivity and thickness of the metal is not uniform.

The coating can best be applied as a plating of copper and the variations in thickness gained in a number of ways. For instance, the brush can be placed in the plating-bath and gradually raised out of it manually or automatically, so that the portions of the brush where a heavy coating is desired would be the longest in the bath; or the brush may simply be arranged in the copper bath with that part which is to have a thick plating nearest the copper electrode; or, again, a plating of uniform thickness could be applied and portions dissolved by acid to gain the desired thinness. The first method is the one I consider preferable.

In Figs. 4 and 5 the old plating of uniform thickness is represented at C, and the jagged lower edge formed by peeling of the coating is shown much as it appears in actual practice. By my improvements this is all avoided and without sacrificing any of the other functions for which such a coating is used. The thin portion of the coating adheres closely and firmly to the carbon and wears away smoothly, while the thick upper portion is sufficient to keep down the resistance of the brush and avoid heating.

I claim—

1. A carbon commutator-brush having a metal coating gradually decreasing in thickness toward the wearing-surface of the brush, for the purpose set forth.
2. A carbon commutator-brush coated with

a plating of copper gradually decreasing in thickness toward the wearing-surface of the brush.

3. A carbon commutator-brush coated with 5 a plating of metal tapering down toward the wearing-surface of the brush until it terminates in practically a mere film, as set forth.

In testimony whereof I have hereto set my hand this 25th day of November, 1890.

EDWIN WILBUR RICE, JR.

Witnesses:

JOHN W. GIBBONEY,  
ELIHU THOMSON.